

D. H. BELLAMORE AND T. I. S. BOAK.  
METHOD OF MAKING PRESSED STEEL VEHICLE WHEELS.  
APPLICATION FILED SEPT. 15, 1919.

1,423,747.

Patented July 25, 1922.

2 SHEETS—SHEET 1.



Fig. 1.



Fig. 2.



Fig. 3.



Fig. 4.



Fig. 5.



Fig. 6.

Fig. 7.

Inventors  
David H. Bellamore  
By their Attorney Thomas I. S. Boak,

Jas. H. Griffin

D. H. BELLAMORE AND T. I. S. BOAK.  
METHOD OF MAKING PRESSED STEEL VEHICLE WHEELS.  
APPLICATION FILED SEPT. 15, 1919.

1,423,747.

Patented July 25, 1922.

2 SHEETS—SHEET 2.



Fig. 8.



Fig. 9.



Fig. 10.

Inventors  
David H. Bellamore  
Thomas I.S. Boak  
By their Attorney  
Jas. H. Griffin.

# UNITED STATES PATENT OFFICE.

DAVID H. BELLAMORE, OF NEW YORK, N. Y., AND THOMAS I. S. BOAK, OF EAST ORANGE, NEW JERSEY, ASSIGNEES, BY DIRECT AND MESNE ASSIGNMENTS, TO STEEL WHEEL CORPORATION, A CORPORATION OF NEW YORK.

## METHOD OF MAKING PRESSED-STEEL VEHICLE WHEELS.

1,423,747.

Specification of Letters Patent. Patented July 25, 1922.

Application filed September 15, 1919. Serial No. 323,836.

To all whom it may concern:

Be it known that we, DAVID H. BELLAMORE, a subject of the King of Great Britain, residing in the city of New York, borough of Manhattan, county and State of New York, and THOMAS I. S. BOAK, a citizen of the United States, residing at East Orange, county of Essex, and State of New Jersey, have invented a certain new and useful Method of Making Pressed-Steel Vehicle Wheels, of which the following is a specification.

This invention relates generally to the art of making disc wheels which are more particularly used with self-propelled vehicles, although manifestly the method of this invention, as well as the resulting product, is adapted for employment in other environments than that specified.

As disc wheels are usually made they are stamped up cold from mild steel such, for example, as ordinary boiler plate. This steel is formed into blanks without any heat treatment whatsoever and immediately subjected to the action of dies while in the cold condition. The material is worked cold through, and the manufacturer depends for the strength of the resulting wheel upon the relatively heavy gage material, since the qualities of the steel employed is such that it is naturally soft and malleable. This procedure is the one carried out in all disc wheels as now manufactured, and as a result of these operations, the product is a wheel of considerable weight. Moreover, the characteristics of the material are such that it cannot be worked cold beyond certain well defined limits, and as a result, the wheels thus far employed have been of most simple conventional form, much less easy riding and aesthetic, than a wooden wheel and far heavier.

With the foregoing considerations in mind, the object of the present invention is to provide a method of making disc wheels which will result in an article of much less weight than disc wheels as heretofore employed, but which will nevertheless, possess strength equal to or greater than the prior wheels. With this object in view, the invention contemplates the manipulation of an alloy steel plate of minimum thickness, heat treated from time to time during the

consecutive operations of its manipulation to render it ductile and finally give a final 55 heat treatment for the purpose of rendering it hard and resilient.

A further disadvantage of disc wheels as now constructed is inherent in the fact that when two discs are secured together in abutting relation with an intermediate cavity or air space between them the construction results in a rapid vibration of the disc when the wheel is passing over a more or less uneven road. This vibration of the disc sets 65 the air between them in rapid vibration, with the result that a noise is produced known in the trade as "drumming." This noise becomes very appreciable when the road is rough and the car is moving at high 70 speed and is disagreeable and undesirable. However, in practically every disc wheel made as described, drumming is common.

Accordingly, a further object of this invention is to provide a method of making a 75 disc wheel which will be entirely devoid of any drumming action and noiseless in this respect.

In carrying out this feature of the invention the space between the two discs of the 80 wheel is adapted to be filled with material for taking up the vibration of the disc, and while this material may vary in substance, we have found that the best results are obtainable from a laminated construction embodying alternate layers or plies made in accordance with felt and balsa wood properly chemically treated to prevent deterioration of the wood and to render it unsusceptible to changes under atmospheric conditions. 90

In the preferred manner of building the wheel of this invention, one of the layers of felt is extended circumferentially to lie between the abutting faces of the opposed 95 disc and form a gasket so that when the discs are secured together by rivets or otherwise, rattling between the adjacent faces of the disc is precluded and a tight joint is formed to keep out the weather. 100

Further features and objects of the invention, both as regards the practicing of the method and resulting article, will be apparent from the foregoing specification and claims, when read in conjunction with 105 the accompanying drawings.

In the accompanying drawings we have illustrated one form of apparatus which may be employed in the carrying out of the method of this invention, but it will be understood that this apparatus is illustrative only, and does not define the limits of the invention.

Figure 1 is a section of two complementary co-operating die members, with which 10 is associated a blank of material to be operated upon thereby;

Figure 2 is a section of the blank as it appears after having been operated upon by the die members of Figure 1.

15 Figures 3 and 4, 5 and 6, are views similar to Figures 1 and 2, but illustrating the manner of forming other portions of the wheel;

Figure 7 is a central section of the parts 20 completed and assembled.

Figure 8 is a section of two cooperating die-members with a laminated filling.

Figure 9 is a section of the compressed blank.

25 Figure 10 is a section of the completed wheel.

The steel from which the wheels of this invention are to be formed, is received from the mill in large sheets which, are in a more 30 or less spotty condition. This term describes the condition wherein certain parts of the steel plate are of a certain degree of hardness, whereas other parts are of entirely different degrees of hardness. This is 35 primarily due to unequal cooling before, during and after the rolling operation, resulting from uneven temperatures and drafts around the rolling mill, while the steel is being rolled. One portion of the 40 plate will be cooled more or less than another portion and when the cooler portion goes under the rolls it will be worked to a greater degree than the warmer portion and thus made harder. If it were attempted to 45 manipulate the material in this condition between the dies, the result would be that the discs produced would be badly warped out of shape and the harder parts of the steel would either be ruptured or, at least, show 50 surface cracks. Accordingly, the first or initial operation in the carrying out of the method consists in heat treating the material for the purpose of normalizing the same.

The steel used in the manufacture of the 55 wheel is an alloy steel, preferably chrome vanadium or, nickel steel, or a high carbon steel. In normalizing this steel the temperature thereof is raised to the normalizing temperature for the particular chemical 60 characteristics of the steel and is maintained at its normalizing temperature for a length of time depending upon the size and shape of the steel, as well as on its chemical characteristics, after which it is removed from 65 the heat and packed in lime, sand or any

other suitable material to insure an even cooling.

At the conclusion of the normalizing operation, the material is blanked in an ordinary press with a conventional blanking punch and die of the size required to give the desired inner and outer diameters of the discs. The blank, from which the main disc is formed, is shown at A' in Figure 1. This blank is of flat, circular shape and, having been normalized, is in the relatively soft, ductile and malleable condition to be properly worked upon by die sections 1 and 2 for manipulating it into the desired shape. The die sections 1 and 2 are complementary 80 and are operated by suitable well known machinery to force them toward one another and to press and work the blank A' into conformity with the complementary sections of the die. As a result of this operation the blank A', after coming from the die sections 1 and 2, partakes of the configuration shown in Figure 2, said blank A' having been formed into the main disc A of the wheel, with the outer circumference of which is 85 integrally formed a portion of the felly of the wheel. The next operation is to stamp out the hub opening a.

The supplemental or reinforcing disc of the wheel is formed from a blank B' shown 90 in Figure 3, by the manipulation of this blank, after the normalizing process, between dies 3 and 4. The dies 3 and 4 press the blank B' into the shape shown in Figure 4 and the hub opening b is thereafter 95 punched in the center of the supplemental disc, so that the resulting supplemental or reinforcing disc B shown in Figure 4 is produced. The blank C' from which the complementary felly section or ring C is 100 formed, is annular in shape, as shown in Figure 5, and after passing through the normalizing process is manipulated by the die sections 5 and 6 to produce the detachable 105 felly section C shown in Figure 6.

It will, of course, be understood that, in practice, the blanks for the respective parts of the wheel are stamped out in quantities from sheet steel, which has been previously normalized and the respective blanks are 110 subsequently transferred to the corresponding machines to be manipulated into the desired shapes.

After the respective parts of the wheel 115 have been manipulated into the desired shapes, such bolt and rivet holes, as are required, are punched out and thereafter the parts of the wheel are subjected to a heat treatment which consists in raising their 120 temperatures to such degree as is necessary 125 to allow of the quenching of the steel in order to obtain the strength and physical characteristics required. This temperature is generally around 1700 degrees Fahrenheit for alloy steel and some where around 1600 130

degrees Fahrenheit for carbon steel. The parts are placed in a furnace capable of retaining its temperature and are maintained at such degree of heat for the required length of time to bring the steel above the critical point, after which the steel is quenched, in a suitable quenching medium, depending upon the chemical constituents of the steel. In practice, the quenching medium may be mineral oil, fish oil, water, brine, or any other suitable material, or any combination of those enumerated. In practice, it is found to be in many instances impractical to simply immerse the parts in the quenching medium, so that it is found preferable, the instant before quenching, to clamp the part to be quenched into a rigid die of the shape and size required to grip it on all sides. While thus maintained in the rigid grip of the die, the parts are quenched and it is found, that when this practice is followed, the parts will maintain the shapes into which they have been manipulated by the forming dies. If the quenching dies are not employed there is a great tendency for the parts to warp and twist.

After the parts have cooled to approximately 200 degrees F. in the quenching medium, they are removed from said medium, and after being placed in a wire rack or basket, are dropped into a tempering bath. The temperature at which this bath will be maintained, and the constituents of the bath are determined by the chemical constituents of the steel to be tempered. For an alloy steel, mineral oil having a high flash point might be used, although a salt bath embodying potassium nitrate and sodium nitrate is found highly efficient. For carbon steel heavy cylinder oil works out very well as a tempering medium. It will be understood, however, that the particular tempering mediums referred to are not exclusive, but are simply enumerated by way of explanation.

After the wheel sections have been maintained in the tempering bath for the correct length of time to insure an even tempering throughout the material thereof, they are removed from the bath and allowed to cool in the air. When cool they are ready for assembling. The parts are assembled as shown in Figure 7, the main disc A and supplemental disc B being preferably secured together by bolts or rivets D, while the main disc A may be provided with suitable fastening bolts or studs after the manner shown in our co-pending application Serial No. 319,129 filed August 22, 1919, for the purpose of holding the detachable section C of the felly in co-operative relation to the permanent portion of the felly forming a part of the main disc. The wheel may be provided with a suitable hub (not shown) or may be simply, provided with bolt holes through which bolts may be

passed for securing the wheel to the conventional form of hub.

It will be noted that the main disc is provided with an annular bead a' extending about the disc exteriorly of the circumference of the supplemental or reinforcing disc B. This bead is formed by the complementary depression and projection 7 and 8 of the die sections 1 and 2 respectively and has, for its function the imparting of radial resiliency to the wheel, after the manner more fully described in the co-pending application Serial No. 319,091 filed August 22nd, 1919.

In carrying out the process of this invention with the dies as shown in the drawings, a wheel structure results which is illustrated in Figure 7, but it will be understood that through the change in shape of the dies, different wheel structures may be formed without departing from the spirit of this invention. The invention does not relate to specific details of the wheel construction, but to the wheel broadly and to the method of making the same. This method consists, speaking generally, in operating upon normalized steel blanks of alloy or high carbon steel, and after the parts have been properly formed in this condition, hardening and tempering said parts. The prior well known methods of making disc wheels, all contemplate the use of mild steel without any heat treatment whatsoever, but when the present method is employed a much superior and lighter wheel results. For concrete example, actual tests have shown that the steel employed in prior wheels, when tested, had a breaking tensile strength of about 64,000 pounds per square inch, whereas the same tests applied to steel treated in accordance with the present invention showed that the steel failed at about 155,000 pounds per square inch, or in other words, that the alloy steel wheel of this invention possesses 250 percent of the strength of the old and well known form of wheel. Moreover, mild steel wheels are generally made of approximately three-sixteenths of an inch stock, whereas the steel of this invention, in order to possess a requisite strength need be made of only one-half that thickness of material. As a comparison between the old and well known form of disc wheels and the wheel of this invention, it is interesting to note that of two wheels possessing the same strength the wheel of the present invention weighs but approximately one-third that of the former wheel. Another important commercial consideration resides in the fact that wheels made from mild steel are non-resilient, and more or less dead, while an alloy steel wheel formed as described, possesses marked resiliency and springy characteristics. Furthermore, the stamping of an

- nular bosses in a mild steel wheel is impractical but is highly practical and advantageous in a resilient steel wheel made in accordance with our method.
- 5 In practicing the method as thus far described a wheel results which embodies two opposed discs with an intermediate air space, and while this wheel possesses all requirements of strength and durability, it is, in a  
 10 measure, open to the objection that where an air space is housed between two disc portions drumming action is very apt to occur when the wheel is traveling rapidly over an uneven road. Accordingly, in its best form  
 15 the wheel is so constructed that the space between the two opposed discs is filled or occupied by a sound-dampening medium intended to take up the vibration of the discs, and, in a great measure to preclude such vibration, to the end that the wheel may be silent under all conditions. The material employed in filling the space in the wheel may differ in substance, but the best results thus far obtained has been through the em-  
 20 ployment of a laminated structure formed of alternate plies of felt and balsa wood. It is desirable that this laminated structure be packed tightly in the space between the discs and in Figures 8 to 10 inclusive of the  
 25 drawings we have shown the consecutive steps of carrying out the method whereby the packing may be properly formed and compressed into a shape to cooperate with the discs, whereby the entire wheel may be  
 30 assembled in an efficient and expeditious manner. In forming the packing a plurality of layers or plies of alternate felt *e* and balsa wood *f* is built up to form a blank after the manner shown in Figure 8, and  
 35 although, manifestly, any number of plies may be employed depending upon the size of the wheel and its thickness through at the hub portion, as well as the thickness of the respective plies. The center ply is prefer-  
 40 ably made of felt and is of a diameter sub-stantially equal to the diameter of the re-enforcing disc *B*, while the remaining plies are made of a lesser diameter equal to the dished portions in the discs *B* and *A*.  
 45 The blank formed as described, is positioned between a pair of cooperating die members 9 and 10, operated upon through suitable pressure mechanism to bring the sections of the die together and compress the  
 50 blank into the form shown in Figure 9, which is the form of the cavity between the opposed discs of the wheel. After the blank has been pressed to the form shown in Figure 9, a central hole *g* is punched out for the hub  
 55 and at the same time additional holes *g'* are

forced through the blank for the bolts which hold the hub to the wheel. When a wheel is to be constructed to embody the packing member just described, the formation of the metallic parts of the wheel is carried out as 70 shown in Figures 1 to 6, but instead of proceeding to assemble as shown in Figure 7, the packing member is assembled between discs *A* and *B* after the manner shown in Figure 10, but it will be noted from this figure that the center ply of the packing member, because of its increased diameter, will extend between the abutting faces of the discs *A* and *B* and form a gasket of relatively soft material so that when the rivets 80 or bolts *D* are put in the discs will not engage with one another, metal-to-metal, but will be cushioned with respect to one another. The riveting of the discs together, will, moreover cause the felt gasket to be 85 compressed with the result that a tight weather-proof joint will be formed at the outer circumference of the reenforcing disc *B*.

The foregoing method of forming and incorporating the filler blank in the wheel is extremely simple and economical to carry out, and the compressing of the blank is conducive to the best results in properly fitting the blank to the space between the discs. 90 In describing this method we have specifically recommended the employment of balsa wood and felt plies, but do not wish to be understood as limiting to this material. We employ them because they are relatively 95 hard and soft, and because balsa wood is very light, and tenacious and when treated chemically is not susceptible to changes under atmospheric conditions. In carrying out the invention, however, other relatively 100 hard and soft materials may be employed, or even material of uniform hardness may be used without departing from the spirit of the invention, which is to be understood as broadly novel as is commensurate with the 105 appended claims.

Having thus fully described the invention, what we claim as new and desire to secure by Letters Patent is:

1. The method of making a disc wheel 115 which consists in manipulating blanks of normalized alloy steel between dies to impart the desired shape thereto, thereafter hardening and tempering the resulting parts and assembling them to form the wheel. 120
2. The method of making a steel wheel which consists in normalizing sheet alloy steel, cutting said steel into blanks, effecting the shaping of the blanks between dies, hardening and tempering the resulting forms 125 and finally assembling them.
3. The method of making a disc wheel which consists in manipulating blanks of normalized alloy steel between dies to impart the desired shape thereto, thereafter harden- 130

ing and tempering the resulting parts, compressing relatively soft and light material into a shape complementary to the shape of the manipulated blanks, and finally assembling the parts with a relatively soft material positioned between the manipulated steel discs. 5

4. The method of making a disc wheel which consists in manipulating blanks of metal to form the discs of the wheel, compressing a non-metallic blank to conform to a portion of the contour of each disc, and assembling the parts with the non-metallic part between the metallic parts. 10

15 5. The method of making a disc wheel, which consists in manipulating blanks of metal to form complementary discs, compressing a laminated non-metallic blank to conform to complementary portions of the contour of the discs, and thereafter assembling the parts with the non-metallic part intermediate the metallic discs. 20

6. The method of making a disc wheel which consists in manipulating metallic blanks to form complementary discs, compressing a non-metallic laminated blank of alternate relatively hard and relatively soft materials into a form complementary to complementary portions of the discs, and thereafter assembling the parts with a non-metallic part intermediate the metallic discs. 25

7. The method of making a disc wheel which consists in manipulating metallic blanks to form complementary discs, compressing a non-metallic laminated blank of alternate layers of felt and wood into a shape to completely fill the space between the complementary portions of the discs when in assembled relation, and thereafter 30 assembling the parts with the non-metallic laminated part intermediate, and filling the space between the discs. 40

8. The method of making a disc wheel which consists in manipulating metallic blanks to form complementary discs, compressing a non-metallic laminated blank into a shape adapted to fill the space between said discs when in assembled relation, and leaving one of the plies of the laminated blank 35 of sufficient size to project circumferentially

of said space, and thereafter assembling the parts with the laminated non-metallic part filling the space between the discs of the wheel and the single ply projecting to form a gasket between the abutting faces of the 55 discs.

9. The method of making a disc wheel which consists in manipulating a flat blank of alloy steel between dies to form said blank into the main disc of the wheel and to 60 form a portion of the felly of the wheel integral with the main disc, then heat treating the disc thus formed to harden and temper the same, manipulating another flat blank of steel to form a reenforcing disc of smaller 65 size than the main disc, then heat treating the reinforcing disc thus formed to harden and temper the same, and thereafter assembling the discs in complementary co-axial relation. 70

10. The method of making a disc wheel which consists in manipulating a flat blank between dies to form said blank into the main disc of the wheel and to form a portion of the felly of the wheel integral with 75 the main disc, manipulating another flat blank of alloy steel to form a reenforcing disc of smaller size than the main disc, and thereafter assembling the discs in complementary co-axial relation, filling the space 80 between the discs with a non-metallic material previously compressed to the shape of the space to be filled.

11. The method of making a steel wheel which consists in manipulating blanks of 85 alloy steel into cooperating shapes between dies, thereafter heat treating the blanks thus shaped to render them resilient, and finally assembling the parts thus produced. 90

12. The method of making a steel wheel which consists in cutting a sheet of alloy steel into blanks, effecting a shaping of the blanks between dies, hardening and tempering the resulting forms, and finally assembling them. 95

In testimony whereof, we sign our names to this specification.

DAVID H. BELLAMORE.  
THOMAS I. S. BOAK.